

May 28, 1935.

P. P. ALEXANDER

2,003,167

APPARATUS FOR FUSING POWDERED MATERIALS

Filed Jan. 9, 1931



Inventor:  
Peter P. Alexander,  
by *Charles E. Tulla*  
His Attorney.

## UNITED STATES PATENT OFFICE

2,003,167

## APPARATUS FOR FUSING POWDERED MATERIALS

Peter P. Alexander, Marblehead, Mass., assignor to General Electric Company, a corporation of New York

Application January 9, 1931, Serial No. 507,709

3 Claims. (CL 219—8)

The present invention relates to a method and apparatus for fusing powdered materials to a relatively soft foundation metal such as steel or iron. In my copending application Serial No.

5 411,634, filed December 4, 1929, now Patent No. 1,971,804 I have disclosed an apparatus and method for spraying a powdered hard metal composition, for example a mixture of tungsten carbide and cobalt heated to an elevated temperature, on to steel. In my prior process the powdered materials are heated by radiation from a carbon heater. However, in certain applications it is necessary to provide a coated article in a short period of time. Under such circumstances 10 the heat radiated by the heater of the prior disclosure may not be sufficiently intense to accomplish the desired result.

To obtain heat necessary to fuse or glaze a hard metal composition in a short period of time, I 20 employ a gas torch of the type disclosed in the copending application of Boris V. Nagashev, Serial No. 477,508, filed August 25, 1930, now Patent No. 1,911,033. A torch of this character produces a long narrow jet of gas sufficiently superheated 25 to melt the cobalt constituent of a hard metal composition such as tungsten carbide and cobalt, in a very short period of time.

The novel features which are characteristic 30 of the present invention are set forth with particularity in the appended claims. The invention itself however will best be understood from reference to the following specification when considered in connection with the accompanying drawing in which the single figure is a view partly in elevation and partly in section of an apparatus whereby my invention may be carried into effect.

Referring more particularly to the drawing, I have indicated at 1, a metal or other suitable framework, on which the apparatus employed in 40 carrying out my invention may be mounted. A gas arc torch 2 is mounted adjacent the base of the framework 1. The torch ordinarily comprises three adjustable tungsten electrodes, two of which, 3 and 4, are indicated on the drawing. The electrodes are connected to a source of 45 alternating current supply through a cable 5.

A capillary or small bore conduit or tube 6 having an outside diameter of about  $\frac{1}{8}$  of an inch and an inside diameter of about 20 mils is centrally disposed with respect to the torch electrodes. Tube 6 is enlarged slightly at point 7 and mounted with the electrodes in an electrically insulating casing 8. An asbestos shield 9 is positioned on the casing 8 adjacent the lower end thereof and is secured thereto by a suitable

refractory cement 10. An elongated conduit 11, similar to conduit 6 and in alignment therewith, is connected to the upper end of the enlargement 7.

The flow of gas issuing from the nozzle of the torch 2 consists of two distinct streams. The inner one issues from the tube 6 and consists of a narrow high velocity gas stream 12 which passes through the arc. This stream comprises superheated gas which transmits the necessary energy from the arc to the glazed or fused surface. In the present apparatus the narrow stream of gas carries the particles of powdered materials which are to be fused or glazed to a foundation metal. To obtain the high velocity, narrow jet of gas, a pipe 13 is connected through a valve 14 to a gas supply pipe 15. Pipe 13 is connected to the tube 11 at the upper end thereof. A mercury gage 16 indicates the gas pressure in the pipe 13.

The second jet of gas issuing from the torch nozzle is a low velocity jet 17 which completely surrounds the high velocity jet 12 and the piece to be glazed. The purpose of the low velocity jet is to provide a shielding atmosphere for the torch electrodes, the central high velocity gas jet and the surface to be glazed. The gas for the low velocity jet is supplied through a pipe 18 which is connected at one end thereof to the gas supply pipe 15 through a valve 19. The other end of the pipe 18 is connected to the inside of the torch nozzle so that the low velocity gas completely fills the space inside the torch nozzle and around the torch electrodes.

A receptacle 20, adapted to contain the powdered materials to be deposited and fused or glazed to a foundation metal is mounted on the framework 1 and at the upper end of tube 11. Receptacle 20 is similar in construction to an ordinary sight feed oil cup. A screw 21, mounted in the upper end of the receptacle, controls the usual feed valve in the receptacle and thereby regulates the feed of powdered materials to the tubes 11 and 6. This feed valve of course can be of any other design which accomplishes the same purpose, that is, the fine regulation of the amount of powdered material supplied to the tubes 11 and 6.

An electrically operated vibrator 22 is positioned on the framework 1 and connected to the upper end of the tube 11 to vibrate the latter and thereby prevent the powdered material from adhering to and becoming packed in the tube.

A pipe 23 connects receptacle 20 with a second mercury gage 24 which indicates gas pressure above the powdered materials in receptacle 20.

Pipe 23 is connected to pipe 13 through a valve 25 so that a desired gas pressure may be maintained above the powdered materials in receptacle 20.

5 An open ended pipe 26 having a valve 27 mounted therein is connected to pipe 23. Before starting operations it is sometimes desirable to blow out the receptacle 20 and the gas pipe 23. This may be accomplished by opening valves 27

10 and 25 for a short time.

In operation, receptacle 20 is filled with powdered materials, for example a mixture consisting of about 87 parts tungsten carbide and 13 parts cobalt. A steel block or other material 28 15 to be surfaced with the material in receptacle 20 is positioned on fire bricks 29 mounted at the lower end of the framework 1 and the gas arc torch 2 placed a suitable distance above the steel block 28. The torch electrodes are then adjusted so that their terminals approach within arcing distance of one another. Vibrator 22 is set in motion and valves 14 and 19 opened to supply hydrogen gas to the torch. An arc is then struck between the torch electrodes. Screw 25 is adjusted to obtain a desired feed of powdered material and valve 25 adjusted so as to obtain a desired gas pressure above the powdered materials in receptacle 20. The torch operates to produce a high velocity narrow jet of 30 superheated gas surrounded by a shielding low velocity jet both of which strike the material to be coated.

The gas from tube 6 is blown out between the electrodes of the torch at high velocity. The gas pressure in front of tube 6 may vary from about 35 one-half to 65-lbs. per square inch, according to the size of the jet and the current in the arc and has sufficient velocity to draw the superheated gases into a narrow, long intense jet.

40 The powdered material fed through pipe 11 and emerging from tube 6 is not melted before it reaches the steel block 28 but is deposited in a powdered condition and then fused thereon. The time required to fuse the powdered material is only a few seconds. The powdered material 45 may be deposited on the steel block 28 either in a single thin layer or in several consecutive layers. The use of successive layers is advantageous since the deposition of such layers insures a product which is substantially free from 50 gas holes.

The deposit obtained by the present process possesses considerable ductility and does not chip off the steel base 28 nor does it crack when heat treated or when severely quenched. The fused 55 deposit may be forged and its homogeneity thereby materially improved. Forging moreover substantially eliminates any voids which may be present in the deposited material.

I have forged a layer of fused material initially consisting of about 13% cobalt and 87% 60 tungsten carbide at a temperature of 950 to 1000° C. At this and higher temperatures the deposited material was relatively soft and the original thickness of the layer was reduced considerably 65 by the forging operation. After forging, the fused layer and supporting steel structure were quenched, while still at a temperature of about 800° C., in cold running water. The quenching operation was given for the purpose of imparting sufficient hardness to the high carbon steel base 28 on which the powdered materials were deposited and fused thereto. The layer of fused material did not crack either during the forging or subsequent quenching.

While I have illustrated my invention in connection with only one powdered composition, it is obvious that the invention is not limited to that particular composition but may be employed equally well in glazing and fusing other powdered compositions. Any change in composition of course imparts different properties to the deposited material. For instance, with higher percentages of refractory carbides the 10 deposits are much harder and less ductile.

15 Although I find it desirable to feed the powdered material through a capillary or small bore tube 6, it is not absolutely necessary to do so. The powdered material may, if desired, be placed on the material to be coated and the torch then applied to the powdered material to fuse it to the foundation metal.

20 Although I prefer to employ a gas-arc torch such as disclosed on the drawing, the invention is not limited to the particular features of construction disclosed. Other forms of torches may be employed if desired provided they supply a non-oxidizing atmosphere and develop the high temperatures necessary for this work.

25 While I prefer to employ hydrogen gas and tungsten electrodes in the torch, the process has been carried out with carbon electrodes and with various gaseous mixtures which are non-oxidizing and non-decarbonizing for example hydrogen with propane, carbon monoxide, hydrogen with 30 nitrogen, and even with substantially pure nitrogen. The monatomic gases such as argon and helium may also be used in this process. If a gas, such as hydrogen, which can be dissociated into its atomic state, is employed, an atomic 35 flame may be formed in which the heat is derived from the recombination of the atoms to form molecules.

35 The deposition and glazing of the powdered materials onto the foundation metal 28 may be 40 carried out continuously or intermittently. If a large surface is to be coated, it is desirable to continuously glaze the surface. However, for glazing small pieces of metal such as the edges of cutting tools, it is preferable in the interests of 45 accuracy and economy to deposit the metal intermittently on the tool edge. The metal 28 may be moved in a horizontal direction under the gas torch in order that any portion of the surface of the metal may be coated. The foundation metal 50 may also be adjusted in a vertical direction.

45 It is sometimes desirable to preheat the foundation metal. Under such circumstances, I connect one phase of the three-phase system indicated at 5 to the metal 28 and the other two phases 55 to the electrodes 3 and 4. These connections are maintained for a few moments only after which the three-phase system is connected to the three torch electrodes as indicated on the drawing. During the preheating operation the material 60 to be fused is fed through the pipe 6 in the same manner as under ordinary operating conditions.

55 I have employed the term "glazing" in the present specification to convey the idea of covering the surface of the foundation metal with 65 a comparatively thin layer of other material which forms a smooth and sometimes shiny surface. This thin layer is not transparent since it consists of an opaque material. Under certain conditions, when the powdered material is deposited intermittently, it is first melted. It then segregates into a large drop on the surface of the foundation metal and spreads over the foundation metal like warm oil over the surface of a piece of ice. If the application of heat is 70 75

stopped at that moment, the material of the top layer preserves its own composition and the fusion zone between the deposited layer and the base metal is limited to a fraction of a mil.

5. What I claim as new and desire to secure by Letters Patent of the United States, is:

1. In combination, a gas arc torch comprising a casing, a plurality of electrodes adjustably positioned relative to one another in said casing, a 10 conduit positioned in said casing to direct a blast of gas between the arcing terminals of said electrodes, means for supplying gas and a powdered composition to said conduit, and means for vibrating said conduit.

10. 2. In combination, a gas arc torch comprising a casing, a plurality of electrodes adjustably positioned to one another in said casing, a capillary conduit positioned in said casing and ar-

ranged to direct a blast of gas between the arcing terminals of said electrodes to thereby produce a narrow superheated jet of gas, means for supplying powdered material and gas to said conduit, means for vibrating said conduit, and means for supplying gas to the nozzle of the torch to provide a shielding atmosphere for said electrodes and said narrow jet.

3. In combination, a gas arc torch comprising a casing, a plurality of electrodes adjustably positioned relative to one another in said casing, a conduit positioned in said casing to direct a blast of gas between the arcing terminals of said electrodes to thereby produce a long narrow gas jet, means whereby a shielding atmosphere may 15 surround said jet, and means for supplying powdered material to said jet.

PETER P. ALEXANDER.